

## UNITED STATES PATENT OFFICE.

JOHN J. MULLIGAN, OF EAST CHICAGO, INDIANA, ASSIGNOR TO UNITED STATES SMELTING REFINING & MINING COMPANY, OF PORTLAND, MAINE, A CORPORATION OF MAINE.

## METHOD OF REFINING METALS.

No Drawing.

Application filed June 19, 1924. Serial No. 721,125.

The invention relates to refining and purifying metals and more particularly to methods involving the use or presence of caustic alkali such as caustic soda in the 5 molten state.

Metal refining methods have heretofore been proposed or used in which molten metal is treated with caustic alkali either alone or mixed with other reagents and in 10 which the impurities rise with the free caustic to the surface of the metal in the form of a more or less fluid dross which must be removed. The molten caustic is a thin and fluid liquid which floats on the 15 surface of the metal bath much as oil floats on water. So long as the covering of caustic is of considerable depth it may be run off without material difficulty but, as its thickness decreases, it is difficult to run it off 20 without running off some of the metal. It is also practically impossible to completely remove the caustic without removing more or less of the metal, since the last of the 25 caustic floats on the metal bath in detached fugitive patches. The molten fluid caustic is also a disagreeable if not a dangerous product to handle since its contact with water may create an explosion with a scattering of caustic through the air and also 30 because its causticity intensifies a burn beyond that due to its heat.

The present invention provides for convenient and complete removal of the dross and molten caustic without removal of the 35 molten metal and also practically eliminates the danger of explosions or burns. This is accomplished by the addition to the floating dross or scum preparatory to its removal of a material which will thicken the molten 40 and fluid caustic and still allow it to float on the metal bath. The thickening material may conveniently be an inert substance having a high melting point which will form with the molten caustic a mixture 45 which is not fluid at the temperature used. Materials of this character which have been successfully used include ordinary building cement, crushed fire brick, crushed lead blast furnace slag, ground commercial fire 50 clay, and sand. A sufficient quantity of a material of this character is scattered over the dross preparatory to its removal and serves to thicken the molten caustic to a 55 pasty mass which may be readily scraped or skimmed from the surface of the bath. By

the addition of an excess of the refractory materials, the scum or dross may be converted into a practically dry powdery mass which may be scraped from the surface of the bath.

While possibly there may be some chemical action between the caustic and some ingredient of the refractory thickening material, as, for instance, between the caustic and the silica of sand, it is believed that the 60 65 principal effect is a physical one which may be considered more as an absorption of the caustic in the material used.

The above method of removing the caustic and drossed impurities from the molten 70 bath may be used in various methods involving a use of caustic which results in its presence in a fluid molten state on the surface of the bath and has been applied with marked advantage in a method of removing 75 arsenic from antimonial lead by treatment with caustic soda which is described and claimed in application No. 678,354, filed Nov. 22, 1923, as a continuation of application No. 579,035, filed August 1, 1922. In 80 this method caustic soda is added to a bath of the molten alloy at a temperature between 900 degrees and 1000 degrees F. and is thoroughly stirred into or mixed with the molten bath, the agitation being continued 85 until the caustic is practically spent, and the dross or scum thus formed is then removed. In applying the present invention to this process, the inert stiffening material is added to the scum or dross preparatory 90 to its removal and, as above explained, mixes with or absorbs the molten caustic forming therewith and with the dross impurities, a pasty or crusty mass which may be readily removed by scraping or skimming and taking with it practically all the 95 fluid caustic without danger and without removal of the metal treated. If the arsenic is removed by successive fractional additions of caustic soda, the addition of the refractory thickening material may be omitted until the final treatment and removal of the final skim, since the presence of free caustics on the surface of the bath after each of the preliminary skims will not be 100 detrimental.

The term "caustic alkali reagent" is intended to include a reagent comprising caustic alkali either alone or mixed with other reagents.

60

65

70

75

80

85

90

95

100

105

110

**What is claimed is:**

1. In a method of refining metals which consists in subjecting molten metal to treatment with a caustic alkali reagent to dross the impurities therein, the addition to the floating dross preparatory to its removal of a material which thickens the fluid caustic therein.
2. In a method of refining metals comprising subjecting molten metal to treatment with a caustic alkali reagent to dross the impurities therein, adding to the floating dross an inert material to thicken the molten caustic therein, and removing the non-fluid mixture thus formed.
3. The method of removing molten caus-

tic and drossed impurities from the surface of a molten metal which consists in absorbing the fluid caustic by the addition of a thickening material and removing the non-  
fluid mixture thus formed.

4. The method of removing arsenic from antimonial lead which consists in treating the molten metal with caustic soda to dross the arsenic, adding to the dross a material which thickens the molten caustic therein, and removing the non-fluid mixture thus formed.

In testimony whereof I have signed my name to this specification.

JOHN J. MULLIGAN.